

A. S. DWIGHT.  
PROCESS FOR TREATING ORES.  
APPLICATION FILED JULY 7, 1913.

1,215,636.

Patented Feb. 13, 1917.

3 SHEETS—SHEET 1.



Witnesses

Witnesses  
A. J. Hybrand

S. Jay Teller

Arthur S. Dingley  
By H. N. Ellis  
Attorney.

1,215,636.

A. S. DWIGHT,  
PROCESS FOR TREATING ORES,  
APPLICATION FILED JULY 7, 1913.

Patented Feb. 13, 1917.



Fig. 3.



Fig. 4.

Witnesses  
H. H. Lybrand  
S. Jay Teller

Inventor  
Arthur S. Dwight  
H. H. Bliss

Attorney

1,215,636.

A. S. DWIGHT,  
PROCESS FOR TREATING ORES,  
APPLICATION FILED JULY 7, 1913.

Patented Feb. 13, 1917.

3 SHEETS—SHEET 3.



Fig. 5.

Witnesses  
H. A. Lybrand  
S. Jay Teller

By

Inventor  
Arthur S. Dwight  
H. A. Bliss  
Attorney

# UNITED STATES PATENT OFFICE.

ARTHUR S. DWIGHT, OF NEW YORK, N. Y., ASSIGNOR TO DWIGHT & LLOYD SINTERING COMPANY, OF NEW YORK, N. Y., A CORPORATION OF DELAWARE.

## PROCESS FOR TREATING ORES.

1,215,636.

Specification of Letters Patent.

Patented Feb. 13, 1917.

Application filed July 7, 1913. Serial No. 777,732.

*To all whom it may concern:*

Be it known that I, ARTHUR S. DWIGHT, a citizen of the United States, residing at New York, in the county of New York and

5 State of New York, have invented certain new and useful Improvements in Processes for Treating Ores, of which the following is a specification, reference being had therein to the accompanying drawing.

10 This invention relates to improvements in the treatment of an ore mass which contains a combustible component, either one united chemically with ore ingredients, or one physically commingled, naturally or artificially, 15 therewith, and from the treatment of which mass products can be obtained that have a value supplemental to the value of the metallic components.

I shall refer to ore masses containing metallic sulfid, but it will be understood that 20 these are to be regarded merely as types of a class any one of which can be subjected successfully to the treatment that I have devised.

25 These sulfid ores have been preliminarily treated by one or another of various methods. The principal characteristic of these is termed "roasting." In the roasting practice that has been most frequently followed 30 the ore, either in the form of native "fines" or as concentrates, is spread on an elongated hearth. While there exposed it is brought to a sulfur-disassociating temperature by the products of combustion of an adjacent fire 35 bed or furnace; and, simultaneously, air is passed in large volumes over the upper surface of the ore.

The streams of air, the products of combustion from the firing furnace and the 40 products of combustion of the sulfid on the hearth are taken together in a miscellaneous gaseous mass through flues to the stacks. Some of the sulfur component is, by the mere action of the heat alone, driven off in 45 the form of a sublimate or fume; much of it is oxidized and forms sulfur gases which are also carried away.

The volumes of air initially supplied have not, heretofore, been, and cannot, economically, be closely controlled. The principal

purpose has been to insure merely that a large volume of air be introduced at the firing end, supplemented by air introduced at points along the hearth, no attempt being made to relate the proportional quantities of the sulfur bodies and the air volumes that finally escape. The chamber below the arch and above the ore is large, relatively, and the quantities of air and gas indiscriminately vary, the air, however, always being largely in preponderance; the aim being, as stated, to insure that a very large amount of air shall be introduced so that there will be assurance that the ore will be properly affected by oxygen without regard to the surplus of air which, as well known, passes, in large volumes, on through the furnace to the stack.

The percentage of the sulfur component of the total gas volume thus carried off in 70 ordinary roasting furnaces is only from one to two per cent., composed partly of sulfur fumes or sublimes and partly of sulfur gases. These gas volumes containing suspended sulfur and sulfur gases, after being 75 taken from the hearth chambers to the stacks, are delivered to the open atmosphere; with exceptional cases that are negligible in comparison with the widely followed practice.

This discharge of the sulfur, although its proportional amount is small in comparison with the total gas volume, is, at all places, objectionable, and now, in many localities, is prohibited.

80 Because the percentage of the sulfur in these volumes of gas, taken away from the ordinary roasters or furnaces, is so low, efforts to neutralize or collect it entail such expense on the treatment of the ore that 90 they are not justified. But, if the percentage of the sulfur can, without increasing the expense of the ore treatment, be raised many times (say from one, or two, per cent. to nine or ten per cent.) the expense incident to 95 their collection is justified, and profit is derived from these by-products supplemental to the profit obtained from the roasted metals.

100 The purpose of the present invention is to

provide a method of treatment, first, whereby the desulfurizing of the ore can be brought closely to the point where the desired predetermined ratio between the metallic components and the residue sulfur in the ore is reached, and, second, whereby the air initially introduced can be accurately regulated in relation to the work of disassociating the sulfur, and the ratio of the air 10 relative to the volumes of sulfur gases and fumes can be accurately controlled, and can be caused to carry off therewith such a proportion of the sulfur that the effort to obtain the sulfur therefrom will be profitable.

15 I first subject to a heating treatment a mass of ore, such as non-roasted ore, which still has a relatively high percentage of a sulfur component, employing, at this stage, air moving, air receiving and air conducting devices whose capacities are predetermined in relation to the sulfur components and in relation to the quantity of air to be utilized in the work. I then take the air 20 (charged with a quantum of the sulfur bodies derived during the first stage) away from the ore and utilize it for the treatment of ore which has been more or less roasted or desulfurized. I cause the air and its contents, during the second stage of treatment, to remove another predetermined amount of the sulfur component, and, second, cause an increase in the amount of sulfur gas in the total gas volume which is taken off after the second stage. I so proportion 25 the various components of the masses and so determine their condition, that after the second stage the proportion of sulfur in the air will be so high that it can be treated profitably in the ways above referred to.

Another object of the invention is to make available, for heat generation, during a later stage of treatment, the non-oxidized sulfur which is obtained as sublimate or fumes during an earlier stage of treatment.

I prefer to produce all the heat necessary for carrying on the steps above mentioned by internal combustion, although it will be understood that more or less of the necessary heat can, at either stage be obtained from external sources. But if the material and the conditions are such as to provide for generating all of the heat by internal combustion, there is greater economy. 50 And if the second, or any later, step of treatment is effected while the ore still contains heat generated by the earlier treatment, there is still further economy. I find it advisable, frequently, to so operate as to have 55 a higher heat generated during the second, or some later, stage than during an earlier one because of the increasing difficulty in disassociating the sulfur after the release initially of the more easily disassociated pro-

portion. And this can be obtained by re- 65 turning the air to its second, or later, stage of work while still highly heated, and, secondly, by so coördinating conditions that the sublimate or fumes of metallic sulfur will, at the second, or later, stage, serve as 70 fuel external to the sulfur still combined with the metal in the ore. More or less of the sulfur initially contained in the native ore can, at discretion, be caused to pass off in such sublimated or fume form during the 75 earlier stage. And sufficient atmospheric oxygen can be delivered in the first instance to provide not only that amount of oxygen which is necessary to perform the predetermined oxidizing work in the earlier stage, 80 but also a surplus amount of oxygen which, when it reaches the second stage of activity, is sufficient to effect the burning or oxidizing of the metallic sulfur which is carried off as sublimate or fume at the first stage; and 85 this can, under proper regulation, be utilized as a course of the high heat required to effect, at the second stage, the further disassociation of more or less of the residue sulfur still combined with the metal. And, of 90 course, this further oxidizing, at the second stage, of the native sulfur component combined with the metal of the ore assists in highly heating the mass at said second stage.

95 Preferably the oxidizing at the second, or later, stage of the free sulfur, drawn away at the first stage, is carried to the point where it is all transformed into a sulfur gas, mainly sulfur dioxid.

With some materials I find it advantageous to separate into two parts the total gas volume derived from the first treatment, one stream carrying the main part of the sublimate or fumed sulfur, and the other stream carrying mainly completely oxidized 100 sulfur. These two streams I regulate and relate to later actions according to conditions. If the conditions are suitable I shunt the stream or volume of gas which is most heavily laden with the sulfur gas (as dioxid) 105 away from the ore which is being subjected to the second treatment, and take it directly to the receiver for the sulfur gas; and take the volume which is charged mainly with free fume sulfur directly to the ore which is to be further desulfurized depending upon 110 its sulfur component for the generation of heat and upon the surplus oxygen in this stream to effect the predetermined oxidizing 115 at the second stage.

120 Another object of the invention is to establish conditions such that not only do I effect, first, the desulfurizing of the ore, and, second, produce a mass of by-product gas which is highly enriched with sulfur, but also, third, deliver the solid ore in the form 125 of sinter blocks or cakes which possess all of the desirable qualities of the sinter that

is now largely manufactured for the blast furnace. And in respect to those phases of the matter which relate to the sintering of the ore, another important object is to prevent the explosions which are liable to occur where the air withdrawn from the ore in the sintering machine is largely charged with oxidizable materials, such as the free sulfur fume, and to prevent the collection of this in the ducts, where it is a serious detriment.

My improved method of treating an ore mass can be carried on with either of several forms of apparatus. In the drawings 15 I have shown some of these.

Figure 1 is a side view of one of the mechanisms;

Fig. 2 is a top plan view of that shown in Fig. 1; 20 Figs. 3, 4 and 5 are, respectively, side views, more or less conventional in character, of other forms of apparatus suitable for this purpose.

In Figs. 1 and 2, A designates, as an entirety, a now well known mechanism adapted for use in roasting ores, and also sintering them. It comprises a track 2 with a series of ore-carrying pallets 3. These are moved slowly in the direction of the arrow 30 a by the usual mechanism, indicated by the wheels at 4. Hoppers 5, or equivalents, feed the ore to the pallets, and 6 indicates an igniter of suitable sort.

After ignition the ore is supplied with 35 air. A suction box 7, a duct 9, an exhaust mechanism 8 and a discharge duct 10 are provided for causing and sustaining internal combustion. These devices are of predetermined capacities in relation to the ore, 40 to its physical conditions, to its sulfur component and to the quantity of air that is to be passed therethrough, all of these varying and requiring regulation.

By properly relating these air moving receiving and conducting devices I succeed, at 45 the outset, in raising to a high percentage the sulfur taken from the ore, and, by selecting and properly co-relating all of the conditions, secure a proportion of sulfur 50 (dioxide and sublimate) approximating five to six per cent. This is in striking contrast with the gas mixture obtained from the ordinary roasting hearths.

This fan 8 is connected by a pipe 10 with 55 a hood 11, arranged over those pallets that are situated between the pallets above the air box 7 and those at the discharge end of the apparatus which are about to deliver their roasted and sintered contents.

60 The air and gases delivered to the hood 11 are caused to pass through the ore contained in the pallets below the hood and into an air box 12, that is connected by pipe 13 with a fan 14 which discharges into a pipe

15, and this in turn delivers to the apparatus, designated diagrammatically at 16, where the gases are treated to utilize the sulfur which they carry.

The hood 11 is so disposed with reference to the path of travel of the pallets 3 that its edges come quite close to the upper edges of the pallets. Thus a close joint permitting practically no leakage of gas may be formed, although this is not necessary because a slight space may, often with advantage, be 75 left between the edge of the hood and the edges of the pallets. This is because, in practice, the amount of gas discharged into the hood 11, which is regulated by the speed of the fan 8, is somewhat less than the 80 amount of gas taken off by the suction caused by the fan 14. It follows from this that some atmospheric air will be drawn under the edges of the hood 11, thus preventing the 85 escape or leakage of any sulfurous gas, which leakage would be objectionable and disagreeable. In the apparatus just described the fans 8 and 14 are suction fans. The gases taken from the wind or air box 7 by the fan 8 will ordinarily contain from 90 two to four per cent. of sulfur dioxide, and more or less, depending upon the character of the ore, elemental sulfur in the form of a sublimate. In these gases there is still 95 sufficient free oxygen to carry on the roasting operations in those pallets or ore receptacles that occupy the space between the hood 11 and the air box 12. The gases taken from the box 12 by the fan 14 and delivered to apparatus 16 are found to be much richer 100 in sulfur dioxide than those taken from the air box 7, the proportion being raised to nine per cent. or more. It is found that, in an arrangement such as shown, the sulfur which passes off into the air box 7 in the 105 form of a sublimate, does not deposit in the pipes 9 and 10, which are relatively short and are maintained at a high temperature, but is delivered into the hood 11 and finally 110 disappears in passing through the ore contained in the pallets below the hood 11, being there oxidized.

In Fig. 3 I have illustrated an apparatus in which are employed non-traveling containers for the ore during the roasting operations. Referring to this view, 17, 17' designate independent ore receivers, each mounted upon trunnions, 18, 18' so as to be free to be inverted, for discharging its contents. Means, either manual or power-operated, may be employed for effecting the inverting operations of these ore containers, such means being typified by the crank handles 19.

Each container has a perforated grate 20, an ore-receiving space 21 above the grate, and an air box or chamber 22 below the grate. The air chamber 22 communicates

with the outside through one of the trunnions 18', which is hollow.

23 represents the fan disposed between the containers 17, 17', connected on one side by 5 pipe 24, with the hollow trunnion 18' of the ore receiver 17, and on the other side, through pipe 25, with a hood 26 that fits closely over the upper end of the ore holder 17'. This hood is movable up and down, 10 the pipe 25 having a slip joint connection to permit this, in order to allow the hood to be lifted to expose the ore receiving portion of the container to allow it to be filled, or to permit the holder as a whole to be tilted for 15 discharging the roasted and sintered ore.

A pipe 27 leads from the hollow trunnion 18' of the ore holder 17' and delivers the gases to a treating apparatus 16, not shown in this view, but similar to that indicated in 20 Fig. 1.

I have not in this view indicated the igniting means for setting fire to the ore at its exposed surface. It will, however, be understood that any suitable form of igniting 25 device may be employed, the igniter or igniters being movable relative to the holders to permit them to be tilted for discharging and to permit the use of the hood 26.

The process as carried out in the apparatus last described is similar to that carried out in the apparatus shown in Figs. 1 and 2. It will be understood that the fan 28 operates to cause air to pass through the body of ore contained in the holder 17 by 35 suction and through the body of ore in the holder 17' by plenum. In using this apparatus the ore in the holder 17' should be ignited before that in the holder 17 is ignited in order that the hood 26 may be brought 40 to place before sulfurous gases are delivered through the pipe 25.

In Fig. 4 I have represented another apparatus by which my invention may be carried out. Here are indicated two apparatus A', A'' similar in general principle to the apparatus illustrated in Figs. 1 and 2, where are employed a series of moving pallets for carrying the ore. In the apparatus A' air is induced to pass through the bodies 50 of ore carried by the pallets 3 by suction induced by a fan 28. The proportions of the apparatus and the speed at which its various parts are moved are so adjusted that a complete roasting and sintering of the 55 ore takes place during the time any particular body or mass thereof is passing the air box 7. In the apparatus A'' the plenum method of forcing the air through the ore is employed, the fan 28 delivering to the hood 60 29. The machine A'' is entirely distinct from the machine A', though the two apparatus are preferably arranged close together so that the length of the ducts between them is reduced as much as possible.

In Fig. 5 I have illustrated another feature of my invention, applied to an apparatus similar in general features to that indicated in Fig. 1, similar reference letters being employed for similar parts in these two views, Figs. 1 and 5.

The air box 7 below the series of pallets nearest the igniter is divided into two chambers, 7' and 7'', by a movable partition 30 arranged to be manually adjusted, as by means of a screw 31.

It is found that the gases passing from the masses of ore nearest the igniter are relatively weak in sulfur dioxid, but contain a relatively large amount of elemental sulfur in the form of sublimate. I therefore connect that chamber of the air box 7 which is below the pallets nearest the igniter, designated 7', with the fan 8, and connect the outlet of this fan with the hood 11, the same as in the apparatus illustrated in 85 Fig. 1. But the chamber 7'' of the air box is connected by a duct 13' with the fan 14, which is also connected with the air box 12 located below those pallets covered by the hood 11. Thus the stronger gases or those 90 containing a larger amount of sulfur dioxid, are delivered directly to the fan 15 and by it to the apparatus 16 where the gas is treated, only part of the gases from the air box 95 7 being delivered to the hood 11 and caused to pass a second time through a body or bodies of ignited and sintering ore, to be freed of the sublimate which they carry, and enriched in sulfur dioxid. In using an apparatus such as shown in Fig. 5 the position of the partition 30 is adjusted to suit 100 the working of the apparatus.

If lead ores are treated according to the process and by means of apparatus such as here described and illustrated, the gases will 105 carry more or less volatilized lead or lead fume. A considerable portion of this will be recovered when the gases pass through a second bed of ignited and sintering ore, the same as it takes up and recovers the sulfur 110 sublimate, as already described; for the semi-fused silicates will absorb and hold whatever load fume comes in contact with them during the passage of the gases. The loss of lead may thus be diminished to a very 115 considerable extent.

I do not in this case claim the novel apparatus herein described, but reserve to myself the right to make that the subject-matter of another application which I propose to file as a division of this case.

What I claim is:—

1. The herein described method of treating sulfid ore for the obtaining therefrom of gas charged highly with sulfur and simultaneously obtaining a uniformly porous sinter, the same consisting in exposing the sulfid ore in a relatively shallow layer or stra- 125

tum, passing air therethrough and causing combustion therein, collecting said air after passing through the ore and while containing a relatively low percentage of sulfur, 5 causing the said combustion to form a uniformly porous sinter body, then passing the said air with its sulfur contents again through the sintered ore and oxidizing more or less of the sulfur residue therein, charging the air volume with the sulfur gases derived therefrom.

2. The herein described method of treating sulfid ores to obtain from them simultaneously with the formation of a porous 15 sinter, a gas rich in sulfur and sulfur products, which method consists in subjecting layers or strata of ore to ignition and supplying combustion-supporting air at two stages thereto after ignition, the air supplied during the second stage being of the same character as that which is delivered to the ore during the first stage.

3. The herein described method of roasting sulfid ores, whereby a porous sinter is obtained together with gaseous products of combustion rich in sulfur content, which consists in arranging ore in shallow layers, igniting it, passing air through said layers to remove or consume sulfur found therein, 25 and collecting and returning said air and the gases of combustion to said ore, in order to complete the burning of the contained sulfur, whereby the gases of combustion thus obtained being charged with sulfur 30 dioxid from the two passages through the sulfur layer, are rich in sulfur products.

4. The herein described method of roasting sulfid ores, whereby a porous sinter is obtained together with gaseous products of 40 combustion rich in sulfur content, which consists in arranging ore in shallow layers, igniting it, passing air through said layers to remove or consume sulfur found therein, and collecting and returning said air and 45 the gases of combustion to said ore while said ore is still hot, in order to complete the burning of the contained sulfur, whereby the gases of combustion thus obtained being charged with sulfur dioxid from the two 50 passages through the sulfur layer, are rich in sulfur products.

5. The herein described method of roasting sulfid ores, whereby a porous sinter is obtained together with gaseous products of 55 combustion rich in sulfur content, which consists in arranging ore in shallow layers, igniting it, passing air through said layers to remove or consume sulfur found therein, and collecting and returning said air and 60 the gases of combustion to said ore while both the ore and the air and gases of combustion are still hot, in order to complete the burning of the contained sulfur, whereby the gases of combustion thus obtained

being charged with sulfur dioxid from the 65 two passages through the sulfur layer, are rich in sulfur products.

6. The herein-described method of treating ore containing a combustible component which consists in arranging said ore in layer 70 form, progressively moving it, igniting it, supplying combustion-supporting air thereto after ignition, subsequently returning the said air at a second stage and again causing it to pass in contact with the ore 75 while the latter is still hot, and collecting the gases generated during the said second stage.

7. The herein described method of treating ore containing sulfur, which consists in 80 arranging said ore in layer form, giving to said ore so arranged a progressive movement, igniting said ore, passing air through said ore in a current, regulated as to speed so as to effect a primary oxidation or sublimation of sulfur, within a defined extent of forward progress of the ore, and returning the air current and the gases therewith and passing them a second time through the 85 progressing layer of ore, whereby an air 90 current laden with sulfur gases in high proportion is obtained.

8. The herein described process which consists in passing more than once through 95 a progressing layer of burning ore, the order of said passages being in the same general directions as that in which the ore moves, a current of air.

9. The process which consists in establishing a moving layer of sulfur-bearing 100 ore, igniting said ore at a given point in its traverse, passing through said ignited and moving layer for a given extent of the traverse a current of an oxidizing agent, whereby by the heat of a reaction, said 105 agent and said ore become heated, and at a further stage in the traverse of the ore layer and while it is still hot passing the same hot current of oxidizing agent through said layer, whereby, owing to the heated 110 conditions specified, the sulfur becomes completely oxidized.

10. The herein described method of treating ore containing sulfur, which consists in arranging said ore in layer form, giving to 115 said ore so arranged a progressive movement, igniting said ore, passing air through said ore within a defined extent of forward progress of the ore, in a current, dividing said current, passing the forward part of said current directly to an apparatus for recovery of the sulfur gases, and passing the rearward part of the current again through a mass of primarily roasted ore.

11. The herein described method of treating ore containing sulfur, which consists in arranging said ore in layer form, giving to said ore so arranged a progressive move-

- ment, igniting said ore, passing air through said ore within a defined extent of forward progress of the ore, in a current, dividing said current, passing the forward part of 5 said current directly to an apparatus for recovery of the sulfur gases, passing the rearward part of the current again through a mass of primarily roasted ore, and conducting the resultant gases and products of combustion to mingle with the gases and prod-

ucts of combustion collected from the forward division of the current, whereby the sulfur may be taken at one operation from both divisions of the current.

In testimony whereof, I have affixed my 15 signature, in presence of two witnesses.

ARTHUR S. DWIGHT.

Witnesses:

HENRY J. STEHLI,

JOSEPH C. BENSON.